

Aug. 14, 1951

A. P. LIEN ET AL

2,564,071

## REFINING OILS

Filed July 2, 1946



Inventors:-  
Arthur P. Lien  
Bernard L. Evering  
Frank W. Haeckl  
By Sam B. Becker  
Attorney

## UNITED STATES PATENT OFFICE

2,564,071

## REFINING OILS

Arthur P. Lien, Hammond, Ind., Bernard L. Ever-  
ing, Chicago, Ill., and Frank W. Haeckl, De-  
troit, Mich., assignors to Standard Oil Com-  
pany, Chicago, Ill., a corporation of Indiana

Application July 2, 1946, Serial No. 681,123

4 Claims. (Cl. 196—13)

1

This invention relates to a novel process of treating hydrocarbon oils. More particularly it relates to a novel process for refining hydrocarbon oils to remove non-hydrocarbon components such as water, inorganic salts, compounds of oxygen, nitrogen and, especially, sulfur and the like. The application of the process of the present invention to hydrocarbon lubricating oil stocks leads to the production of high viscosity index (V. I.) lubricating oils containing substantially no inorganic components and a reduced or negligible content of low V. I. aromatic hydrocarbons.

It is known to refine hydrocarbon oils by treatment with liquid hydrogen fluoride, as described, for example in British Patent 292,932. It is also known to refine hydrocarbon oils with solutions of  $\text{BF}_3$  in liquid hydrofluoric acid, as described for example in United States Letters Patent 2,343,841. However, the prior art processes suffer from certain disadvantages. We have discovered that unexpected advantages and results can be obtained by treating hydrocarbon oils in sequence with hydrogen fluoride and with liquid  $\text{HF-BF}_3$ .

We have found that liquid hydrogen fluoride has a relatively limited capacity to increase the viscosity index of any given lubricating oil stock. Also, although liquid hydrogen fluoride is a fairly efficient solvent for sulfur compounds contained in hydrocarbon oils, it appears that certain sulfur compounds such as high molecular weight mercaptans, for example n-dodecyl mercaptan, exhibit little or no solubility in liquid hydrogen fluoride at ambient temperatures.

Although liquid  $\text{HF-BF}_3$  is an extremely active desulfurizing agent for hydrocarbon oils, the  $\text{BF}_3$  component thereof is quite expensive and is readily converted by water to inactive  $\text{BF}_3$  hydrates from which the  $\text{BF}_3$  can be recovered only indirectly and at great expense and difficulty. Since most unrefined hydrocarbon oils normally contain a not inconsiderable quantity of water, the direct application of liquid  $\text{HF-BF}_3$  thereto is unduly expensive and must be preceded by a dehydration operation which adds to the expense of the refining process. Most hydrocarbon oils contain some sulfur compounds which are readily removable by less powerful reagents than liquid  $\text{HF-BF}_3$  and at considerably less expense. It is, therefore, desirable, in view of the high relative cost of liquid  $\text{HF-BF}_3$ , to segregate readily removable sulfur compounds from hydrocarbon oils by a less expensive reagent and to reserve the employment of liquid  $\text{HF-BF}_3$  for difficultly removable sulfur compounds.

In the treatment of hydrocarbon lubricating oil stocks for the purpose, inter alia, of increasing viscosity index, the direct application of liquid  $\text{HF-BF}_3$  to the stock causes very substantial treating losses due in part to the fact that the  $\text{HF-BF}_3$  or the  $\text{HF-BF}_3$  extract exhibits undesirable solvent capacity for high V. I. paraffinic components

2

of lubricating oil stocks. As a result, the direct application of liquid  $\text{HF-BF}_3$  to lubricating oil stocks leads not only to aggravated losses due to excessive extraction, but also to products of lower viscosity index than those which can be obtained by the process of this invention, as will be described hereinafter.

We have found that the treatment of hydrocarbon oils with hydrogen fluoride followed by treatment of the resultant partially refined oils with liquid  $\text{HF-BF}_3$  avoids the disadvantages associated with the employment of these treating agents alone.

It is an object of this invention to provide a novel process for the treatment of hydrocarbon oils, which process comprises contacting said oils with hydrogen fluoride, separating partially refined hydrocarbon oils from the products of the hydrogen fluoride treatment and thereafter continuing the refining of said partially refined oils by contacting them with liquid  $\text{HF-BF}_3$ .

Another object of this invention is to provide a novel and economical process for the removal of water, unsaturated hydrocarbons and low V. I. aromatic hydrocarbons, and compounds of sulfur and nitrogen from hydrocarbon oils, in which process a hydrocarbon oil containing one or more of the aforesaid undesirable constituents is intermingled or contacted with liquid hydrogen fluoride, the resultant mixture is then separated into two liquid layers, viz. a partially refined hydrocarbon oil layer and a hydrogen fluoride extract layer which contains impurities removed from the hydrocarbon oil, and the partially refined hydrocarbon oil is thereafter intermingled with liquid  $\text{HF-BF}_3$  to effect the substantially complete removal of impurities.

A further object of this invention is to provide a process for treating hydrocarbon lubricating oil stocks in sequence with liquid hydrogen fluoride and liquid  $\text{HF-BF}_3$  to produce lubricating oils of higher viscosity index than could be obtained by the application of either reagent alone, which process is accompanied by unexpectedly low treating losses.

An additional object of this invention is to provide a process for refining hydrocarbon oils with liquid  $\text{HF-BF}_3$  in the presence of low-boiling saturated hydrocarbons, whereby cracking of said hydrocarbon oils is inhibited or substantially eliminated.

In the first stage of the process of this invention the hydrocarbon charging stock is partially refined by being intimately contacted with hydrogen fluoride. The general temperature range within which contacting with hydrogen fluoride is feasible lies between about 0° F. and about 450° F. Ordinarily, it is desirable to effect contacting under sufficient pressure to maintain both the hydrocarbon charging stock and most, if not substantially all, of the hydrogen fluoride in the liq-

uid phase. However, this is not to be taken as the invariable rule, for there are some instances in which hydrogen fluoride vapor may be applied to a liquid or liquefied hydrocarbon charging stock to effect partial refining thereof. For example, we have observed that if hydrogen fluoride vapors are passed into a sulfur-containing hydrocarbon oil, the oil absorbs hydrogen fluoride and, in time, a liquid layer containing hydrogen fluoride and sulfur compounds settles from the oil, leaving a supernatant raffinate oil of reduced sulfur content.

As will be shown hereinafter, contacting of a hydrocarbon oil with liquid hydrogen fluoride at temperatures above about 200° F. results in appreciable cracking, as evidenced by the production of hydrocarbons boiling below the initial boiling point of the charging stock. It is believed that when the extent of cracking is limited, for example to about 20 weight per cent of the charging stock or less, the low V. I. constituents of the oil are selectively cracked. Cracking is accompanied by condensation of low V. I. aromatic hydrocarbons having relatively low solubility in liquid HF to polynuclear aromatic hydrocarbons which are readily soluble in liquid HF and are therefore extracted by the HF. Cracking of the low V. I. constituents of hydrocarbon oils is accelerated by the concurrent employment of temperatures between about 200° F. and about 450° F., preferably between about 300° F. and about 450° F., and relatively large volumes of hydrogen fluoride, e. g., 50, 100 or even 200 volume per cent or more of liquid hydrogen fluoride based on the volume of the hydrocarbon charging stock.

The quantity of hydrogen fluoride which will be applied in the first step of our process will be dependent to some degree on the nature of the hydrocarbon charging stock and on the degree of refining which is being sought. However, a generally applicable range comprises a liquid hydrogen fluoride volume between about 5 per cent and about 100 per cent, based on the volume of the hydrocarbon charging stock being treated, although an even larger volume of hydrogen fluoride, e. g., 200 volume per cent, may sometimes be desirable.

The contacting between the hydrogen fluoride and hydrogen charging stock may be effected in conventional equipment constructed of hydrogen fluoride-resistant materials. As a general rule, hydrocarbons are substantially immiscible with liquid hydrogen fluoride and are of lower density. Accordingly, liquid hydrogen fluoride lends itself readily to counterflow contacting with hydrocarbon oils. Ordinarily, contacting between the hydrogen fluoride and the hydrocarbon charging stock may be effected by counterflowing the charging stock and liquid hydrogen fluoride in a tube or tower which may, if desired, be packed with hydrogen fluoride-resistant spacing materials to cause intimate contacting between the two streams. The contacting tower may be operated in such fashion that it contains a major amount of hydrogen fluoride or of the hydrocarbon charging stock. When the contacting tower is operated rich in hydrogen fluoride, the hydrocarbon charging stock may be introduced into the liquid hydrogen fluoride phase and will ascend therethrough and will ultimately leave the contacting tower at or about its top. In this case the hydrogen fluoride phase becomes rich in extracted materials, e. g., sulfur compounds and/or low V. I. aromatic hydrocarbons, and the extract

layer itself can operate as a solvent to promote better refining of the charging stock.

It should be understood that the process of this invention is not limited to particular means or methods for effecting contact between hydrogen fluoride and the hydrocarbon charging stock. Other methods of contacting than those described above may be employed, such as concurrent flow of charging stock and hydrogen fluoride, mechanical stirring, orifice mixing and settling, etc. Regardless of the method of contacting, a multiplicity of contactors may be employed.

The efficiency of contacting and of the subsequent separation of extract and raffinate layers is markedly affected by the viscosity of the hydrocarbon charging stock. It is desirable, especially when viscous hydrocarbon oils are employed as charging stock, to add diluents such as light hydrocarbons to reduce the viscosity. These diluents serve not only to improve the efficiency of the first stage contacting and separation operations, but serve additionally to repress excessive cracking of the charging stock in the second stage of the process of this invention. The diluents which are employed may be recovered from the refined charging stocks and recycled. It may be desirable to employ as a diluent a crude light hydrocarbon stock, e. g., a sulfur-containing naphtha which may itself be refined concurrently with the refining of a more viscous hydrocarbon charging stock.

The time of contacting will depend to some extent on the other reaction variables which are employed, the nature of the hydrocarbon charging stock and the degree of refining sought to be effected. Ordinarily, we may employ contacting periods between about 1 and about 360 minutes or even more, if desired. In order to repress excessive cracking which might otherwise ensue at temperatures above about 200° F., especially when relatively large hydrogen fluoride:oil ratios are employed, it is desirable to limit the contacting to a period less than about 180 minutes, preferably between about 5 and about 150 minutes.

In a preferred mode of operation the hydrocarbon charging stock is subjected to a preliminary treatment with 5 or more volume per cent of liquid hydrogen fluoride at ambient temperatures, e. g. about 50° F. about 100° F., to remove readily extractable materials. Following the extraction operation, a raffinate consisting of partially refined oil is separated from extract phase comprising extracted materials dissolved in or combined with liquid hydrogen fluoride. The raffinate may then be contacted with liquid HF-BF<sub>3</sub>, upon which a partial pressure of BF<sub>3</sub> is superimposed but is preferably first contacted with liquid hydrogen fluoride at elevated temperatures between about 200° F. and about 450° F. in order to effect further refining, conversion and selective cracking of low V. I. constituents of the charging stock. The treatment at elevated temperature is followed by a contacting or settling period with liquid hydrogen fluoride at ambient temperatures. If desired, the elevated temperature contacting operation may be effected directly on the hydrocarbon charging stock without subjecting the same to preliminary extraction with liquid hydrogen fluoride at ambient temperatures. We have observed that the greater the V. I. improvement obtained in the hydrogen fluoride treating step, the greater is the overall V. I. improvement which is obtained in the two-stage treating process of this invention. Accordingly, it is extremely desirable to select the

operating conditions in the hydrogen fluoride treating stage to obtain a very substantial increase in the viscosity index of the charging stock, e. g. to employ temperatures between about 200° F. and about 450° F. concurrently with the employment of about 50 volume per cent or more of hydrogen fluoride, based on the volume of hydrocarbon charging stock.

Upon completion of the contacting of hydrogen fluoride and the hydrocarbon charging stock, the resultant mixture or emulsion is separated into a partially refined hydrocarbon oil and a liquid hydrogen fluoride extract layer. Where contacting between hydrogen fluoride and oil has been effected at high temperatures, e. g. 200° F. or more, the hydrogen fluoride may be distilled or flashed from the contacting mixture and this hydrogen fluoride may thereafter be recovered by condensation. This method of hydrogen fluoride removal, however, necessitates the subsequent extraction of the partially refined or converted hydrocarbon oil with 5 to 100 volume per cent or more of liquid hydrogen fluoride to remove the conversion products formed in the oil, preferably at ambient temperatures of 100° F. or less, e. g. room temperature. Hydrogen fluoride may be recovered from the extract phase by conventional methods, such as distillation, and reused. There is no necessity for removing small amounts of dissolved or suspended hydrogen fluoride from the partially refined hydrocarbon oil, as this oil will be subjected in the second stage of our process to contacting with liquid HF-BF<sub>3</sub>.

Ordinarily, upon completion of the contacting operation between the hydrogen fluoride and hydrocarbon oil, the resultant mixture or emulsion is brought to a temperature such that the hydrogen fluoride and partially refined oil can be readily separated as distinct liquid phases by settling, centrifuging or similar operations. Usually temperatures below about 150° F. are used in the separation step and it is desirable to effect separation at about room temperature. In order to facilitate the separation, especially where viscous hydrocarbon oils are involved, it is desirable to add a light liquid or liquefied hydrocarbon diluent to the mixture of oil and hydrogen fluoride, e. g., propane, butane, pentane, paraffinic or cycloparaffinic naphthas or the like.

Following the separation operation, the diluent can be removed from the partially refined oil, usually simply by distillation. However, it is desirable to retain a hydrocarbon diluent in the partially refined oil throughout the second stage treatment of the oil with liquid HF-BF<sub>3</sub>. HF-BF<sub>3</sub> is a much more powerful cracking catalyst than hydrogen fluoride alone under similar conditions and the inclusion of light paraffinic hydrocarbons, either formed in the hydrogen fluoride contacting operation or added to the partially refined oil, in the oil being contacted with HF-BF<sub>3</sub> tends to repress excessive cracking thereof.

In the second stage of our process, the partially refined hydrocarbon oil derived from the first stage, with or without complete separation of the hydrogen fluoride therefrom, is contacted with liquid HF-BF<sub>3</sub> in quantity sufficient to form a distinct liquid phase under the contacting conditions. The amount and composition of the liquid HF-BF<sub>3</sub> which are employed will be dependent upon the extent of refining sought to be effected. Generally, we may employ between about 5 and about 100 per cent by volume of liquid HF-BF<sub>3</sub>, based on the volume of oil being contacted therewith, although the employment of even larger

volumes of liquid HF-BF<sub>3</sub> may sometimes be desirable. The BF<sub>3</sub> concentration in the liquid HF-BF<sub>3</sub> may vary between about 1 and about 200 per cent by weight, based on the weight of hydrogen fluoride. We prefer to employ between about 10 and about 60 per cent by weight of BF<sub>3</sub>, based on the weight of hydrogen fluoride, and have carried on desirable operations with between about 15 and about 25 per cent by weight of BF<sub>3</sub>.

10 A wide range of temperatures is available for effecting the refining of hydrocarbon oils with liquid HF-BF<sub>3</sub>, viz. temperatures between about -30° F. and about 350° F. However, liquid HF-BF<sub>3</sub> is a powerful cracking catalyst and is capable of effecting a considerable amount of conversion of hydrocarbon lubricating oil stocks to lower boiling hydrocarbons even at room temperature. Since uncontrolled cracking of the partially refined oil charged to the second step of 15 our process tends to reduce the yield of finished oil, we prefer to employ temperatures below about 100° F., particularly temperatures between about 40° F. and about 80° F., during the contacting thereof with liquid HF-BF<sub>3</sub>.

20 Sufficient pressure is maintained on the contacting mixture in the second stage of our process to obtain essentially liquid phase contacting. However, BF<sub>3</sub> is extremely volatile and, depending upon the temperature and the BF<sub>3</sub> concentration in the liquid contacting mixture, considerable BF<sub>3</sub> pressure may be generated in the contacting zone.

25 We may employ contact times between about 1 and about 180 minutes in the second stage contacting operation, preferably between about 5 and about 120 minutes. When liquid HF-BF<sub>3</sub> is employed at preferred temperatures falling between about 40° F. and about 80° F., we prefer to employ contact times between about 5 and 30 about 120 minutes.

35 By the inclusion of cracked hydrocarbon products derived from the first stage operation of our invention, by the deliberate addition of low boiling hydrocarbons to the charging stock, or both, by maintaining temperatures below about 100° F., 40 by employing between about 10 and about 60 per cent by weight of BF<sub>3</sub> based on the weight of hydrogen fluoride and by limiting the duration of 45 contacting, cracking of the charging stock may be inhibited or satisfactorily controlled in the second stage operation of our process to yield refined oils of high viscosity index in good yields.

50 The contacting methods and equipment employed in the second stage of our process are essentially the same as those employed in the first stage. Because of the relatively high volatility of BF<sub>3</sub>, it will be desirable to employ equipment capable of withstanding moderate pressures, even when the temperature employed in the second 55 stage is 100° F. or less.

60 If the second stage contacting operation has been effected at temperatures substantially above 100° F., the contacting mixture is preferably cooled to a temperature below 100° F. before effecting separation of refined oil and liquid HF-BF<sub>3</sub> therefrom. In a preferred method of 65 operation, the second stage contacting mixture is cooled to a temperature between about 0° F. and about 80° F. and the cooled mixture is then centrifuged or allowed to stratify under the influence of gravity into two liquid layers of different density, viz. an HF-BF<sub>3</sub> extract layer containing materials extracted from the oil and a supernatant raffinate. The HF-BF<sub>3</sub> can be recovered from the extract layer by conventional 70 75

methods, e. g., distillation, and reused in the contacting operation.

Hydrogen fluoride and  $BF_3$  may conveniently be recovered from the raffinate layer by stripping with heat, with or without the aid of stripping agents. These stripping agents may be any inert gas, hydrocarbon gas or vaporized light liquid. Alternatively,  $HF-BF_3$  may be removed from the raffinate by passage thereof in contact with metal fluoride salts such as  $NaF$   $CaF_2$  or the like, optionally supported upon spacing materials such as activated alumina or carbon. Metal fluoride salts combine with hydrogen fluoride and  $BF_3$  to form complex salts from which the adsorbed or reacted hydrogen fluoride and  $BF_3$  can be recovered by heating. Fluoride impurities may also be removed from the raffinate by washing with water or dilute alkalies, treatment with sulfuric acid, or passage of the raffinate over dehydrogenating metal oxides, e. g., chromium oxide supported on alumina, bauxite, etc.

The refined oil may be clayed, acid-treated or, if oils of special properties are desired, may be further extracted with conventional solvents such as Chlorex (B,B'-dichlorodiethyl ether), phenol, furfural, nitrobenzene or the like. It is usually desirable to adjust the initial boiling point of the refined oil by distillation.

In order to illustrate the novel two-stage treating process of this invention, reference is made to the accompanying flow diagram which is a schematic representation of one embodiment.

By way of example and not with the intention of limiting the invention, the processing of a hydrocarbon lubricating oil stock to improve V. I. will be described. By the operation of the two-stage process of this invention on lubricating oil stocks sulfur, oxygen and nitrogen compounds and water are removed from the stock, together with low V. I. constituents. A hydrocarbon lubricating oil stock from the source 10 is passed by pump 11 into heat exchanger 12 wherein it is brought to the desired temperature, which may be the processing temperature employed in the hydrogen fluoride contacting zone. From heat exchanger 12 the charging stock passes through line 13 into a hydrogen fluoride contacting zone 14, which has been schematically represented in the form of a tower, although it will be readily understood that other contacting means, as indicated above, may be employed instead. Contacting tower 14 may be provided with mechanical agitating means (not shown). In order to facilitate contacting and the subsequent settling operation, it is desirable to add a light hydrocarbon diluent to the charging stock by means of valved line 13A. Suitable light hydrocarbon diluents include liquid propane, butanes, pentanes, hexanes, saturated naphthas and the like. In tower 14 the charging stock is intimately contacted with liquid hydrogen fluoride in quantity sufficient at least to maintain a distinct liquid phase under the contacting conditions, viz., usually between about 5 and about 100 per cent by volume of liquid hydrogen fluoride, based on the volume of charging stock. Ordinarily it is preferred to use commercial, substantially anhydrous hydrogen fluoride. The hydrogen fluoride enters the contacting tower through line 15 or through lines 15 and 16. If desired, liquid hydrogen fluoride may be introduced into the tower at a number of other vertically spaced points. As shown, the charging stock is introduced at a low point in the contacting tower, preferably below the level of the hydrogen fluoride extract phase, with the result

that the hydrogen fluoride is used very efficiently, since the extract is presented for further contact with additional charging stock which is thereby extracted to some extent and at the same time strips occluded paraffinic materials from the extract. If desired, tower 14 may be partially or substantially completely packed with spacing materials which are resistant to the action of the mixture being contacted.

Although temperature between about 0° F. and about 450° F. may be employed in contacting tower 14, it may be desirable to use temperatures between about 200° F. and about 450° F. Sufficient pressure will be maintained in the contacting tower to maintain essentially liquid phase contacting conditions. Depending on the nature of the charging stock, the extent of V. I. improvement which is sought and the temperature employed, the time of contact in tower 14 may vary between about 1 and about 360 minutes. We prefer to effect a very substantial increase in the V. I. of the lubricating oil stock in tower 14 and to this end we prefer to employ temperatures between about 200° F. and about 450° F. therein and contact times between about 5 and about 180 minutes. Under these conditions partial selective cracking and extraction of low V. I. constituents of the charging stock are effected; far greater increases in V. I. are obtained under these conditions than are obtainable at temperatures below 200° F. The temperature in contacting tower 14 may be controlled by controlling the temperatures of the charging stock and hydrogen fluoride streams introduced therein and, if desired, by additional temperature adjusting means such as heating and cooling jackets or coils (not shown).

A partially refined lubricating oil stock passes overhead from contacting tower 14 through line 17, pressure-reducing valve 18 and thence to heat exchanger 19 wherein its temperature is suitably adjusted to maintain a desired temperature in settler 21. From heat exchanger 19, the oil passes through line 20 to settler 21. It is desirable to employ settling temperatures below about 150° F., preferably below about 100° F., e. g. about 75° F. in settler 21. A light hydrocarbon diluent may be introduced into settler 21 through lines 22 and 23, in lieu of or in addition to the diluent which may be introduced into contacting tower 14 through line 13A. In settler 21 the mixture of hydrocarbons and liquid hydrogen fluoride derived from contacting tower 14 is allowed to stratify under the influence of gravity into two liquid layers. The more dense liquid hydrogen fluoride layer is withdrawn from settler 21 through line 23 and forced by pump 24 into valved line 16 and/or valved line 25 to line 15 for recycle to contacting tower 14.

The lighter, partially refined hydrocarbon oil layer flows over weir 26 and is removed from settler 21 through line 27, whence it is forced by pump 28 into the second stage contacting zone. It is not necessary to strip the small proportion of hydrogen fluoride dissolved or dispersed in this oil, usually between about 0.5 and 2 weight per cent hydrogen fluoride, before subjecting the oil to the second stage treating operation of this invention. Settler 21 is provided with a valved vent line 27A through which light hydrocarbon gases which may be produced by cracking in tower 14 or by partial vaporization of light hydrocarbon diluents introduced into the system at line 13A and 22 may be separated. Light gases removed through line 27A usually contain some hydrogen fluoride which may be re-

covered by absorption, as will be described hereinafter.

In contacting tower 14 there is formed an extract phase comprising water, compounds of oxygen, sulfur and nitrogen, and low V. I. materials which have been removed from the hydrocarbon charging stock, dissolved in liquid hydrogen fluoride. The extract layer is withdrawn from the bottom of contacting tower 14 through valved line 29 and is introduced into a stripping zone 30 to remove hydrogen fluoride which is present in the extract layer in the free state or in loose chemical combination with the extracted materials. Stripper 30 can be operated at temperatures between about 100° F. and about 190° F., preferably about 100° F. to about 160° F. at pressures between about 5 and about 50 p. s. i. g., preferably at about atmospheric pressure. Under these conditions free or loosely bound hydrogen fluoride is vaporized from the extract layer and passes from the top of stripper 30 through line 31, valved line 32 and condenser 33 to the hydrogen fluoride storage tank 34.

The denuded extract layer which contains some hydrogen fluoride in firm combination, apparently in chemical combination, is withdrawn from the bottom of stripper 30 through valved line 35 and is passed into hydrogen fluoride regeneration zone 36. In the regeneration zone, the denuded extract is subjected to temperatures between about 200° F. and about 500° F., preferably about 250° F. to about 350° F. at about atmospheric pressure, although if desired, somewhat higher pressures may be employed. Under these conditions, tarry extract materials are partially decomposed to regenerate hydrogen fluoride which vaporizes and passes overhead from the regeneration zone through line 37, whence it may be passed into line 32. Extract materials are removed from regeneration zone through 40 valved line 38.

Hydrocarbon charging stocks usually contain small, but nonetheless appreciable amounts of water which are absorbed by the liquid hydrogen fluoride in contacting tower 14 and, because of the repeated (recycle) use of hydrogen fluoride, tend to concentrate in and dilute the hydrogen fluoride. Consequently, it is necessary intermittently or continuously to subject a portion of the hydrogen fluoride to dehydration. This may be done by passing hydrogen fluoride vapors from lines 31 and 37 through valved line 39 into an azeotropic distillation tower 40 wherein a maximum boiling hydrogen fluoride-water azeotrope is separated as a liquid phase from substantially anhydrous hydrogen fluoride vapors which pass overhead through lines 41 and 42 to hydrogen fluoride storage tank 34. The liquid hydrogen fluoride-water azeotrope is withdrawn from tower 40 through valved line 43 and may be removed from the system. Anhydrous hydrogen fluoride may be regenerated from this azeotrope by known methods, for example by treatment with fluorosulfonic acid. Also the hydrogen fluoride-water azeotrope, which is still an active dehydrating agent, may be contacted with the charging stock which is introduced into contacting tower 14 in order to dry the same.

Referring now to the schematic representation of the second stage treating operation of the process of this invention, partially refined oil derived from the first stage treating operation is transferred from settler 21 into line 27 and forced by pump 28 through heat exchanger 44 into a low point of the second stage contacting

zone 45 which, like the first stage contacting zone, is represented in the form of a vertical tower. Tower 45 may be unpacked or partially or wholly packed with solid spacing materials 5 resistant to the action of the mixture being contacted. The oil is preferably introduced below the level of the extract phase in tower 45. Liquid HF-BF<sub>3</sub> is introduced into tower 45 at a plurality of vertically spaced points through lines 46, 47 and 48. Fresh anhydrous HF may be introduced into tower 45 by lines 93, 93' and 46. In tower 45 the oil and liquid HF-BF<sub>3</sub> streams are intimately contacted and counterflowed. A substantial amount of the BF<sub>3</sub> is introduced by line 48 to tower 45.

A temperature between about -30° F. and about 350° F. is maintained in tower 45. The contacting temperature may be controlled by controlling the temperatures of the various streams which are introduced into tower 45 and/or by temperature-control jackets or coils (not shown). Because of the capacity of liquid HF-BF<sub>3</sub> to induce catalytic cracking of hydrocarbons at relatively low temperatures, we prefer to employ a contacting temperature below about 100° F., preferably between about 40 and about 80° F., in tower 45. Sufficient pressure is maintained in tower 45 to obtain essentially liquid phase contacting conditions, although a considerable BF<sub>3</sub> vapor pressure, e. g., about 100 p. s. i. or even more, is permissible.

The quantity of HF-BF<sub>3</sub> which is introduced into tower 45 is sufficient to develop and maintain a distinct liquid HF-BF<sub>3</sub> extract phase in the lower portion of the tower, the solute of said extract phase comprising low V. I. constituents derived from the oil being processed, sulfur compounds and the like.

The time of contact will be dependent upon other reaction variables which are selected and upon the extent of refining and V. I. improvement sought to be effected. Ordinarily the oil is contacted for a period of time between about 1 and about 120 minutes.

Upon completion of the contacting operation refined oil containing dissolved and dispersed hydrogen fluoride and BF<sub>3</sub> flows overhead from tower 45 through line 49 and pressure reducing valve 50 into heat exchanger 51. In heat exchanger 51 the refined oil stream is cooled to a suitable settling temperature and is then passed into settler 52, which is depicted as an inclined gravity settler, although it should be understood that equivalent means such as centrifuges may be used. In settler 52 a lower layer of liquid hydrogen fluoride containing dissolved boron fluoride settles out and is removed for recycle to tower 45 by line 47 and pump 47A. Refined oil, which is of lower specific gravity than the liquid hydrofluoric acid solution flows over weir 53 into the upper portion of settler 52. Settler 52 is provided with a valved vent line 54 through which BF<sub>3</sub>, usually contaminated with low boiling diluent hydrocarbons such as methane, ethane, propane, etc. derived from cracking or introduced into tower 45 as diluents, can be vented. It is desirable to recover BF<sub>3</sub> from the low boiling hydrocarbon gases which are vented by line 54, suitably by the employment of an absorption operation which will be described hereinafter. Refined oil passes from settler 52 through valved line 55 into BF<sub>3</sub> stripping tower 56 provided with a heating coil 57 and a dephlegmating coil 58. In tower 56, BF<sub>3</sub> and small amounts of low boiling hydrocarbons vaporize from the refined oil

to pass overhead through line 59, whence  $\text{BF}_3$  can be recycled to tower 45 through valved line 48. In order to prevent the accumulation of inert gases in the contacting system it is desirable intermittently or continuously to divert a portion of the gas stream passing through line 59 through valved line 60 for recycle (by lines not shown) to the  $\text{BF}_3$  absorber 90. The refined oil which contains small amounts of dissolved or dispersed hydrogen fluoride, and possibly low boiling hydrocarbons boiling at room temperature or higher at atmospheric pressure, is transferred from stripper 56 by valved line 61 and pump 62 into a hydrogen fluoride stripping tower 63 provided with heating coil 64 and dephlegmating coil 65. In tower 63, the hydrogen fluoride is stripped from the refined oil usually as an azeotrope with low boiling hydrocarbons and passes overhead through line 66 and condenser 67 into settler 68, wherein a lower liquid hydrogen fluoride layer forms and is removed by valved line 69 for recycle to hydrogen fluoride storage tank 34 (by lines not shown). Light hydrocarbons are removed from settler 68 by valved line 70 and may, if desired, be recycled as a diluent through lines 13A or 22. Gases may be vented from settler 68 through valved line 71. A refined oil which is essentially free of all but traces of fluorides is removed from the hydrogen fluoride stripper 63 through valved line 72 and may be subjected to such after-treatment as may be desired.

The liquid  $\text{HF-BF}_3$  extract phase which settles to the lower portion of tower 45 is withdrawn through valved line 73 and passed into extract stripper 74. In stripper 74 dissolved and loosely bound  $\text{HF}$  and  $\text{BF}_3$  are vaporized by the application of heat, for example through heating coil 75, and pass overhead through line 76. Suitable temperatures for use in stripper 74 are about 100° F. to about 190° F., preferably between about 100 and 160° F. The partially denuded extract is removed from the base of stripper 74 through valved line 77 and is forced by pump 78 into regenerator 79 provided with a heating coil 80 or other heating means. In regenerator 79 the extract is subjected to temperatures sufficient to release hydrogen fluoride and  $\text{BF}_3$  which are firmly, probably chemically, bound to the materials extracted from the hydrocarbon oil which was processed in tower 45. The liberated hydrogen fluoride and boron fluoride leave regenerator 79 by valved line 81. The hydrogen fluoride and  $\text{BF}_3$  in lines 76 and 81 can be passed through valved line 82 into fractionator 83 wherein liquid hydrogen fluoride is separated as bottoms and transferred through valved line 84, pump 85 and lines 42 and 32 to hydrogen fluoride storage tank 34.  $\text{BF}_3$ -containing gases leave tower 83 through valved line 86 and may be recycled to tower 45 via line 48, together with fresh  $\text{BF}_3$  which is introduced into the system via valved line 87. All or part of the  $\text{BF}_3$  may be diverted from line 86 through valved line 88 and cooler 89 for passage to absorber 90.

Hydrogen fluoride and  $\text{BF}_3$  from lines 76 and 81 may be passed through valved line 91 for recycle to tower 45 through line 48. All or part of the stream passing through line 91 may be diverted through valved line 92 into line 88 for passage to absorber 90.

In absorber 90,  $\text{BF}_3$ -containing streams derived from various points in the treating system (for example in lines 54, 76, 81 and 86), more or less contaminated with low boiling hydrocarbons,

are subjected to absorption in liquid hydrogen fluoride. For this purpose liquid hydrogen fluoride, which is introduced into storage tank 34 through line 93, is passed through valved line 94 and cooler 95 into the upper portion of absorber 90. Suitable operating conditions in the absorber are temperatures between about 40 and about 150° F. and pressures between about 10 and about 500 p. s. i. The cold, liquid hydrogen fluoride selectively absorbs the  $\text{BF}_3$  from the  $\text{BF}_3$ -containing gas streams and a solution of  $\text{BF}_3$  in liquid hydrogen fluoride is withdrawn from the base of absorber 90 through valved line 96, whence it may be recycled by pump 97 in line 98 to valved line 99, pump 100 and heat exchanger 101 to line 46 for recycle to tower 45. In order to adjust the  $\text{HF:BF}_3$  ratio of the stream in line 99, liquid hydrogen fluoride may be admitted thereto from storage tank 34 and line 94. Part or all of the  $\text{HF-BF}_3$  solution withdrawn from the base of absorber 90 may be passed by lines (not shown) to the  $\text{HF-BF}_3$  fractionator 83. Unabsorbed gases such as methane, ethane, propane, etc. are vented from the top of absorber 90 through valved line 102 and may be removed from the system or recycled, wholly or in part, as diluents through lines 13A and/or 22.

Following are examples of the application of the process of this invention to Mid-Continent lubricating oil stocks of S. A. E. 20 and 50 grades. In the runs presented hereinafter the oil to be refined and liquid hydrogen fluoride or liquid  $\text{HF-BF}_3$  were intermittently contacted in a carbon steel stirring bomb whose contents were agitated at about 1725 R. P. M. by a mechanical stirrer. The bomb was provided with a bleed-off tube terminating at a point well above the level of liquid hydrogen fluoride or  $\text{HF-BF}_3$ , allowing ready removal of supernatant raffinate from the lower extract phase. In all runs on S. A. E. 20 grade stock, the hydrogen fluoride was employed in the amount of 515 cc. per liter of oil. In the runs on the S. A. E. 50 grade stock, a solution containing 70 volume per cent of the oil in normal pentane was prepared and the solution was treated with hydrogen fluoride in the amount of 515 cc. per liter of oil and, where indicated, with  $\text{BF}_3$  in addition. Where no amount of  $\text{BF}_3$  is indicated in the following table, the oil was contacted with hydrogen fluoride alone. The S. A. E. 20 lubricating oil stock which was charged contained about 0.66 weight per cent sulfur in the form of various organic sulfur compounds and the S. A. E. 50 grade lubricating oil stock contained 0.71 per cent by weight of sulfur. As a result of our treating process, substantially all the sulfur was removed from these oils.

In the following table, runs entitled A and B or A, B and C denote sequential treatments of the charging stock and the raffinate or raffinates produced therefrom, the hydrogen fluoride:charging stock volume ratio being maintained constant throughout the series of refining operations. Where sequential operations were effected upon the oils, cracked products were not removed between the treating steps.

The amounts of cracked products were determined by vacuum distillation of a sample of the refined oil to remove hydrocarbons boiling below the initial boiling point of the charging stock. It is well-known that the cracking of high molecular weight hydrocarbons always produces both lower boiling and higher boiling hydrocarbons than the charging stock. It will be apparent

therefore, that the amount of cracking was actually greater than the figures in the following table indicate.

Where treating operations were effected at temperatures above room temperature, upon completion of contacting, the contacting mixture was allowed to cool to room temperature and stirred for 30 minutes at about 1725 R. P. M. at that temperature before allowing the contacting mixture to stratify into raffinate and extract layers.

An inspection of run 1 of the table shows that treatment of the charging stock with liquid HF-BF<sub>3</sub> at about room temperature produced a surprising amount of cracking, viz. nominally 7.4 weight per cent on the charging stock, and that the relatively low V. I. of 92 was obtained at the relatively high treating loss of 54.1 per cent based on the weight of the charging stock. The specific dispersion of the product, being below 100, indicates substantially complete removal of aromatic hydrocarbons from the charging stock. From this run it appears that HF-BF<sub>3</sub> is an extremely good solvent for aromatic hydrocarbons. It appears, however, that the aromatics react to form an HF-BF<sub>3</sub>-aromatic complex which exhibits solvent capacity for some of the relatively high V. I. constituents of the charging stock. Although we do not choose to be bound by this theory, it deserves some confidence because of the experimentally observed high treating loss and because, as will be brought out more fully hereinafter, hydrogen fluoride pre-treatment at 212° F. or 330° F. to remove the bulk of the aromatics

tained in run 2 but that this loss was offset by a substantial gain in V. I., from 95.4 in run 2 to 98.6 in run 3. The combination of hydrogen fluoride treatment at room temperature and at 330° F. to yield an oil having a V. I. of 94.7, as shown in runs 3A and 3B represents about the maximum V. I. which we have been able to obtain by hydrogen fluoride treatment alone of this particular charging stock.

It will be apparent from the runs discussed above that the combination of hydrogen fluoride and HF-BF<sub>3</sub> treatment of the hydrocarbon lubricating oil stock produced an unpredictable and unexpected result, viz. a high V. I. product which could not be obtained with either hydrogen fluoride treatment alone or with HF-BF<sub>3</sub> treatment alone. Moreover, this result was obtained at no expense in the yield of finished product; rather, the combination treating process produced an increased yield of higher V. I. oil. It will be noted that the specific dispersions of the products of runs 2 and 3 indicate that substantially complete removal of aromatics from the charging stock was effected by the treatments. This fact coupled with the fact of far lower treating losses than the one obtained in run 1 indicates that in run 1 the HF-BF<sub>3</sub>-aromatic complex apparently retained solvent properties for high V. I. paraffinic constituents of the oil.

Run 4 indicates that our novel combination treating process can be applied to S. A. E. 50 grade oil to produce high V. I. products without exaggerated treating losses.

Table

| Run No. | BF <sub>3</sub> , g./l. | Time, Hrs. | Temp., °F. | Vis., 100° F. | Vis., 210° F. | V. I. | Color, N. P. A. | n <sub>D</sub> <sup>20</sup> | D <sub>4</sub> <sup>20</sup> | Spec. Disp. | Cumulative Treating Loss, Wt. Per Cent |          | Total | Yield, Vol. Per Cent |
|---------|-------------------------|------------|------------|---------------|---------------|-------|-----------------|------------------------------|------------------------------|-------------|----------------------------------------|----------|-------|----------------------|
|         |                         |            |            |               |               |       |                 |                              |                              |             | Extraction                             | Cracking |       |                      |

## REFINING OF MID-CONTINENT S. A. E. 20 GRADE LUBRICATING OIL STOCK

|       |     |    |     |     |      |      |      |        |       |     |      |      |      |      |
|-------|-----|----|-----|-----|------|------|------|--------|-------|-----|------|------|------|------|
| Feed. |     |    |     | 594 | 60.4 | 55.5 | 8    | 1.5087 | 0.914 | 131 | 46.7 | 7.4  | 54.1 | 48.7 |
| 1.    | 121 | 1½ | 81  | 321 | 52.9 | 92.0 | 1½-2 | 1.4761 | 0.860 | 99  |      |      |      |      |
| 2A.   |     | 3  | 212 | 427 | 56.3 | 76.7 | 4-4½ | 1.4942 | 0.890 | 119 | 17.2 | 3.3  | 20.5 | 81.6 |
| 2B.   | 84  | 1½ | 42  | 312 | 52.8 | 95.4 | 1-1½ | 1.4782 | 0.865 | 100 | 35.4 | 5.7  | 41.1 | 62.2 |
| 3A.   |     | 1¼ | 76  |     |      |      |      |        |       |     | 15.0 |      | 15.0 | 86.5 |
| 3B.   |     | 3  | 330 | 317 | 53.0 | 94.7 | 4    | 1.4840 | 0.874 | 107 | 25.7 | 12.7 | 38.4 | 64.5 |
| 3C.   | 85  | ½  | 76  | 281 | 51.4 | 98.6 | 2½-3 | 1.4764 | 0.859 | 98  | 31.7 | 13.3 | 45.0 | 58.6 |

## REFINING OF MID-CONTINENT S. A. E. 50 GRADE LUBRICATING OIL STOCK

|       |     |    |     |       |       |      |    |        |       |     |      |     |      |  |
|-------|-----|----|-----|-------|-------|------|----|--------|-------|-----|------|-----|------|--|
| Feed. |     |    |     | 4,006 | 149.0 | 52.1 | 8  | 1.5214 | 0.910 | 121 | 25.8 |     | 25.8 |  |
| 4A.   |     | 1¼ | 80  | 2,115 | 118.6 | 75.6 | 4½ | 1.5033 | 0.910 | 121 |      |     |      |  |
| 4B.   |     | 3  | 212 | 1,855 | 112.9 | 79.7 | 7  | 1.5022 | 0.894 | 121 | 30.1 | 1.4 | 31.5 |  |
| 4C.   | 115 | ½  | 76  | 947   | 85.0  | 94.0 | 2  | 1.4820 | 0.867 | 101 | 50.0 | 4.5 | 54.5 |  |

from the charging stock resulted in much lower treating losses for a given extent of the V. I. improvement.

An inspection of run 2 in the above table shows that treatment of the charging stock with liquid hydrogen fluoride at 212° F. followed by low temperature treatment of the resultant raffinate with liquid HF-BF<sub>3</sub> resulted in the relatively low total loss of 41.1 weight per cent and the relatively high V. I. of 95.4, as compared with the results obtained in run 1.

In run 3 the charging stock was extracted with liquid hydrogen fluoride at room temperature, the resultant raffinate was treated with liquid hydrogen fluoride at 330° F., followed by a contacting and separation period at about room temperature, and the resultant raffinate was then treated at room temperature with liquid HF-BF<sub>3</sub>. It will be noted that this three-stage treatment resulted in a slightly increased treating loss over that ob-

55 The application of the process of this invention to the manufacture of high V. I. lubricating oils has been emphasized. However, the process is far more generally applicable, for example, for the refining of diverse crude liquid hydrocarbons such as are obtainable from petroleum by fractionation or conversion, from shale oil, coal or coal tar hydrogenation, and the like. Suitable hydrocarbon charging stocks which may be processed in accordance with this invention include naphthas, kerosenes, Diesel oils, gas oils, furnace oils, range oils and the like. Our process is, in fact, generally applicable to the refinement of hydrocarbon oils containing one or more of the following: unsaturates, aromatics, compounds of oxygen, nitrogen or sulfur.

70 An especially advantageous application of the process of this invention, in addition to its application to the refining of hydrocarbon lubricating oil stocks, can be made to white oil or mineral oil stocks.

Another especially advantageous application of our process may be made to sulfur-containing oils, especially to relatively heavy oils such as furnace oils. If doctor-sweet products are desired, oxidizing agents such as  $\text{SO}_2$ ,  $\text{SO}_3$ , oxygen, air, nitrogen oxides, nitric acid and the like may be introduced into the first stage contacting zone wherein liquid hydrogen fluoride and oil are intimately commingled.

A substantial proportion of the sulfur in hydrocarbon oils can be eliminated as hydrogen sulfide by treating such oils concurrently with liquid hydrogen fluoride and hydrogen. A hydrogen partial pressure between about 50 and about 3000 p. s. i. g., preferably about 200 to about 2000, may be employed. Increased hydrogenation may be effected by employing a nickel liner in tower 14. When hydrogen is employed, we prefer to use temperatures between about 150° F. and about 500° F. preferably about 250° F. to about 400° F.

We claim:

1. The process for refining a hydrocarbon lubricating oil stock having a specific dispersion in substantial excess of 100, which process comprises contacting said stock with about 50 per cent by volume of liquid hydrogen fluoride, based on the volume of said stock, at a temperature of about 200° F. under pressure sufficient to maintain the liquid phase, for a period of time sufficient to effect a substantial increase in the viscosity index of said stock, cooling the resultant mixture of liquid hydrogen fluoride and lubricating oil stock to a temperature below about 100° F., separating a partially refined lubricating oil stock and a liquid hydrogen fluoride-containing phase, thereafter contacting said partially refined lubricating oil stock with liquid hydrogen fluoride-boron fluoride containing between about 10 per cent and about 60 per cent by weight of boron fluoride, based on the weight of the hydrogen fluoride, at a temperature between about 40° F. and about 80° F. under a pressure sufficient to maintain the liquid phase, the quantity of hydrogen fluoride-boron fluoride being sufficient at least to form a distinct liquid phase under the contacting conditions, and separating a refined hydrocarbon oil having a specific dispersion not in excess of about 100 hydrogen fluoride-boron fluoride from the resultant mixture.

2. The process for refining a hydrocarbon lubricating oil stock having a specific dispersion in substantial excess of 100, which process comprises contacting said stock with about 50 per cent by volume of liquid hydrogen fluoride, based on the volume of said stock, at a temperature of about 330° F. under pressure sufficient to maintain the liquid phase, for a period of time sufficient to effect a substantial increase in the viscosity index of said stock, cooling the resultant mixture of liquid hydrogen fluoride and lubricating oil stock to a temperature below about 100° F., separating a partially refined lubricating oil stock and a liquid hydrogen fluoride-containing phase, thereafter contacting said partially refined lubricating oil stock with liquid hydrogen fluoride-boron fluoride containing between about 10 per cent and about 60 per cent by weight of boron fluoride, based on the weight of the hydrogen fluoride, at a temperature between about 40° F. and about 80° F. under pressure sufficient to maintain the liquid phase, the quantity of hydrogen fluoride-boron fluoride being sufficient at least to form a distinct liquid phase under the contacting conditions, and separating a refined hydrocarbon oil having a specific dispersion not in excess of about 100 hy-

16  
drogen fluoride-boron fluoride from the resultant mixture.

3. A process of refining a hydrocarbon lubricating oil stock having a specific dispersion in substantial excess of 100, which process comprises contacting said stock with liquid hydrogen fluoride at a temperature between about 50° F. and about 100° F. under pressure sufficient to maintain the liquid phase, the quantity of hydrogen fluoride being at least sufficient to form a distinct liquid phase under the contacting conditions, separating the resultant mixture into a liquid hydrogen fluoride-containing phase and a first raffinate lubricating oil stock having a specific dispersion in substantial excess of 100, thereafter contacting said first raffinate lubricating oil stock with liquid hydrogen fluoride at a temperature between about 200° F. and about 450° F. under a pressure sufficient to maintain the liquid phase, cooling the resultant mixture to a temperature between about 50° F. and about 100° F. and then separating the same into a liquid hydrogen fluoride-containing phase and a second raffinate lubricating oil stock having a specific dispersion in excess of 100, contacting said second raffinate lubricating oil stock with liquid hydrogen fluoride-boron fluoride at a temperature between about 50° F. and about 100° F., under pressure sufficient to maintain the liquid phase, the quantity of said liquid hydrogen fluoride-boron fluoride being sufficient at least to form a distinct liquid phase under the contacting conditions, and separating a refined lubricating oil having a specific dispersion not in excess of 100 and a liquid phase comprising principally hydrogen fluoride-boron fluoride from the resultant mixture.

4. A process for refining a hydrocarbon lubricating oil stock having specific dispersion in substantial excess of 100, which process comprises contacting said stock with between about 50 and about 200 percent by volume of liquid hydrogen fluoride at a temperature between about 200° F. and about 450° F. under pressure sufficient to maintain the liquid phase, separating the resultant mixture at a temperature between about 75° F. and about 150° F. into a liquid phase comprising principally hydrogen fluoride and a second liquid phase consisting essentially of a partially refined lubricating oil stock having a specific dispersion less than the specific dispersion of said hydrocarbon lubricating oil stock but in excess of 100, thereafter contacting the partially refined stock with between about 5 and about 100 volume percent of liquid hydrogen fluoride-boron fluoride containing between about 10 and about 60 percent by weight of boron fluoride at a temperature between about 40° F. and about 80° F. under pressure sufficient to maintain the liquid phase, and separating from the resultant mixture a refined lubricating oil having a specific dispersion not in excess of about 100 and hydrogen fluoride-boron fluoride.

ARTHUR P. LIEN.  
BERNARD L. EVERING.  
FRANK W. HAECKL.

#### REFERENCES CITED

The following references are of record in the file of this patent:

#### UNITED STATES PATENTS

| Number    | Name       | Date          |
|-----------|------------|---------------|
| 2,343,744 | Burk ----- | Mar. 7, 1944  |
| 2,343,841 | Burk ----- | Mar. 7, 1944  |
| 2,378,762 | Frey ----- | June 19, 1945 |
| 2,405,995 | Burk ----- | Aug. 20, 1946 |

**Certificate of Correction**

Patent No. 2,564,071

August 14, 1951

**ARTHUR P. LIEN ET AL.**

It is hereby certified that error appears in the printed specification of the above numbered patent requiring correction as follows:

Column 3, line 49, for "hydrogen" read *hydrocarbon*; column 4, line 49, before "about" insert *to*; column 5, line 55, for "HE-BF<sub>3</sub>" read *HF-BF<sub>3</sub>*; column 8, line 4, for "extracted" read *extracted*; line 74, for "gases" read *gases*; columns 13 and 14, in the table, under the heading "*n<sub>D</sub><sup>20</sup>*", opposite "Run No. 3B" for "1,4840" read 1.4840; under the same heading, opposite "Run No. 4A" for "1,5033" read 1.5033; same column, opposite "Run No. 4B" for "1,5022" read 1.5022; same column, opposite "Run 4C" for "1,4820" read 1.4820; same table, under the heading "*D<sub>4</sub><sup>20</sup>*" opposite "Run No. 4B" for "0,894" read 0.894; same column, opposite "Run No. 4C" for "0,867" read 0.867; column 15, lines 48 and 75, respectively, after "100" insert *and a liquid phase containing*;

and that the said Letters Patent should be read as corrected above, so that the same may conform to the record of the case in the Patent Office.

Signed and sealed this 20th day of November, A. D. 1951.

[**SEAL**]

**THOMAS F. MURPHY,**  
*Assistant Commissioner of Patents.*